

# UNITED STATES PATENT OFFICE.

MELVIN H. HUBBARD, OF UTICA, NEW YORK.

## PROCESS FOR ELIMINATION OF COLORING-MATTER FROM PAPER-STOCK.

977,013.

Specification of Letters Patent. Patented Nov. 29, 1910.

No Drawing.

Application filed April 9, 1910. Serial No. 554,518.

*To all whom it may concern:*

Be it known that I, MELVIN H. HUBBARD, a citizen of the United States, residing at Utica, in the county of Oneida and State 5 of New York, have invented certain new and useful Improvements in Processes for Elimination of Coloring-Matter from Paper-Stock, of which the following is a specification.

10 This invention relates to improvements in processes for the elimination of coloring matter from paper-stock in the conversion of the same into pulp; and an object of this invention is to provide a simple, reliable and 15 efficient process of the character described.

Another object of this invention is to provide a process of the character described which will result in the production of pulp which will be thoroughly cleansed of all 20 impurities, which will be sanitary and hygienic in character, which will possess body and in which the original fiber of the paper-stock will be preserved.

A third object of this invention is to provide a process of the class referred to which will result in the production of pulp having great density.

My new process is particularly well-adapted to the elimination of ink and other 30 coloring matter from newspaper stock in the conversion of the same into pulp; but it is not limited to this specific use.

My invention is carried out as follows: The paper-stock, which may consist of old 35 newspapers, books and like printed matter, is placed in a beating engine of the ordinary type and is there beaten up fine. The temperature of the mixture of stock and water in the beating engine is raised, during the 40 time the stock is being subjected to the beating operation, to between eighty degrees and one hundred and twenty degrees, Fahrenheit. After the stock has been beaten up fine, and has been reduced to the consistency 45 of pulp, the following solution is added, namely: Ten (10) parts of soap; twenty (20) parts of whiting; and seventy (70) parts of water. The pulp is now beaten until this solution has thoroughly permeated 50 every portion of the mass and has thoroughly removed and separated the coloring matter, ink and carbon from the particles of paper-stock constituting the body portion of the pulp. The coloring matter, ink and

carbon are then partially washed away by 55 the introduction of clear water into the beating engine. To wash the mass thoroughly free from the separated coloring matter, ink and carbon, the pulp is now run from the beating engine into a vat provided with a 60 suitable agitating apparatus by which the mass is kept constantly stirred and moving in the vat. The latter is filled from time to time with clear water and this water is then drawn off, thereby washing the mass. 65 This operation of refilling with clear water and drawing off the water is repeated as often as may be necessary to remove the impurities from the stock. It will be understood by all those skilled in this art that, if 70 necessary, more than one washing vat may be used in order to rid the stock thoroughly of the carbon particles and other impurities; and, if the amount of coloring matter in the original stock be small or if time be deemed 75 not an essential factor, the washing vat may be entirely dispensed with and the entire washing be carried out in the beating engine.

To the now thoroughly-washed pulp is added a solution consisting of one part of 80 commercial chlorid of lime and three parts of water and this solution is thoroughly mixed with the pulp by means of the agitating apparatus with which the washing vat is equipped; or, if the mixing be done in the 85 beating engine, the mixing will result from the operation of the ordinary beater-roll. After the pulp is thoroughly bleached, it is again rinsed or washed with clear water, until it is thoroughly clean. The pulp will 90 now be found to be free from disease germs and to be of a clear white color and will be adapted for use in making paper or any article to the manufacture of which paper pulp may be adapted. To make paper, the 95 washed mass is emptied into a chest; and, after being mixed with wood sulfite, it is run through a Jordan engine and then out upon a paper machine, in the ordinary manner. If a grayish color is desired, the washing process will, of course, be stopped before 100 all the ink and carbon particles are removed and a less quantity of the chlorid solution will be used.

While I prefer to use, as a bleaching 105 agent, chlorid of lime, other well-known bleaching agents may be substituted therefor without departing from the spirit of my

invention; thus, a ten per cent. solution of sulfuric acid may be used.

While I have herein specified certain definite proportions in which the ingredients enter the solutions hereinbefore mentioned, yet it will be understood that these exact proportions may be varied without departing from my invention.

In using the term, soap, herein I desire to be understood as including the ingredients which ordinarily are used to form a soap; that is, an alkali and a fat acid. And it is immaterial whether the soap be prepared before its mixture with the whiting or the latter be added to the soap-making ingredients.

I claim:

1. The process of removing coloring matter from paper-stock, which consists in reducing the latter to pulp; treating the pulp with a compound consisting of soap and an earth mixed in water; and then bleaching.
2. A step in the process of removing coloring matter from paper-stock, which consists in reducing the latter to pulp; and treating the pulp with a compound consisting of soap and whiting mixed in water.
3. The process of removing coloring matter from paper-stock, which consists in reducing the latter to pulp; treating the pulp

with a compound consisting of soap and an earth mixed in water; and then adding a solution of chlorid of lime.

4. The process of removing coloring matter from paper-stock, which consists in reducing the latter to pulp; adding to the pulp a mixture of soap, whiting and water; washing the pulp thus treated; and finally adding a bleaching agent.

5. The process of removing coloring matter from paper-stock, which consists in reducing the latter to pulp; adding to the pulp a mixture of soap, an earth and water; washing the pulp thus treated; and finally adding a bleaching agent.

6. The process of removing coloring matter from paper-stock, which consists in reducing the latter to pulp; adding to the pulp a mixture of soap, whiting and water; washing the pulp thus treated; and finally adding a solution of chlorid of lime.

In testimony whereof I hereunto set my hand this eighth day of April, 1910, at New York city, N. Y., in the presence of the two undersigned witnesses.

MELVIN H. HUBBARD.

Witnesses:

JAMES HAMILTON,  
EMMA I. McCARTHY.